

Nov. 22, 1932.

H. J. STEHLI

1,888,296

SINTERING MACHINE PALLET

Filed Jan. 20, 1930

Fig. 1.



Fig. 2.

INVENTOR.  
H. J. Stehli  
R. F. Bourne  
ATTORNEY.

## UNITED STATES PATENT OFFICE

HENRY J. STEHLI, OF CEDAR GROVE, NEW JERSEY

## SINTERING MACHINE PALLET

Application filed January 20, 1930. Serial No. 422,220.

Heretofore, in order to strengthen iron castings, and particularly with comparatively thin sections that have to withstand shock and strain, a reinforcing member, such as an ordinary steel or iron bar or rod, has been placed in the mold before the iron for the casting has been poured therein, to embed the bar in the resulting casting. It has been found that ordinary carbon steel rods or bars, 5 embedded in the iron castings, crystallize and become brittle, doubtless due to the sudden heating of the rods or bars by the enveloping molten cast metal and the gradual cooling thereof, hence such rods or bars become use- 10 less in the castings for the purposes of a reinforcement.

The object of my invention is to produce reinforced metal castings that will have increased strength as compared to the strength 20 of an unreinforced casting of the same metal.

In carrying out my invention I place in a mold a reinforcing member, such as a rod or bar, that will not become crystallized from the heat of the molten metal poured around 25 it, and pour molten metal into said mold to embed said member, and I allow the casting containing said member to cool in the mold.

I have discovered that a nickel steel member embedded in a cast metal during the casting does not become crystallized and does not 30 lose its original strength, but its strength rather becomes increased and said member greatly increases the strength of the casting compared with such a casting minus said 35 member.

For some purposes I place a nickel steel rod in a mold as a reinforce and pour molten iron into the mold to embed said rod in the casting, and I allow the casting to cool. The 40 nickel steel alloy becomes heat-treated from the heat of the molten metal embedding it in such a way that the rod becomes greatly increased in tensile strength with a non-crystalline structure, with the result that the casting 45 containing the rod becomes practically

unbreakable for the uses intended, by reason of the presence of such rod.

While the percentage of nickel in the steel rod or member may be variable for the desired casting, I find that a nickel steel rod 50 including steel of any desired composition having from 3% to 5% of nickel therein when used as a reinforcing member in cast iron becomes non-crystalline and has increased 55 strength.

My improvement may be used in various relations where strong metal castings are desired, and the same is particularly useful in making pallets for sintering machines which contain heated ores while traveling on tracks. 60

In the accompanying drawing Fig. 1 is a plan view of a pallet for a sintering machine, and Fig. 2 is a section on line 2, 2, in Fig. 1.

The numeral 1 indicates an iron casting in 65 the form of a pallet for a sintering machine embodying my improvement, wherein the nickel steel reinforcing rod 2 is embedded in and in contact with the casting. This is accomplished by placing the rod in the mold for the casting and pouring the molten iron into 70 the mold around the rod to embed the rod in the casting in contact with the cast metal, after which the casting containing the rod is allowed to cool in the mold. By reason of the 75 heat of the molten metal of the casting 1 embedding the rod 2 the tensile strength of the latter becomes greatly increased, the rod does not become crystallized and the casting becomes practically unbreakable in the use for 80 which it is made. My improved pallet is

capable of withstanding repeated heating and cooling to which it is subjected in the process of sintering ores contained in the pallet as well as shocks incident to discharging sintered ores from the pallet and operation of the same in a sintering machine, during which uses the rod does not become crystallized and the strength of the casting and its durability 85 is increased.

Having now described my invention what I claim is:

1. A sintering machine pallet comprising a cast iron body containing one or more nickel steel reinforcing rods embedded therein, said rods containing less than 5% of nickel.
- 5 2. A sintering machine pallet comprising a cast iron body containing one or more nickel steel reinforcing rods embedded therein, said rods containing between three and five per cent of nickel.

HENRY J. STEHLI.

15

20

25

30

35

40

45

50

55

60

65